

Nov. 10, 1936.

W. T. REDDISH

2,060,529

METHOD OF REMOVING SERICIN FROM SILK

Original Filed Sept. 21, 1933

Mahogany Sulphonates

C

The soap and mahogany together constitutes a suspending and emulsifying agent superior to either alone, and together sulfonilizes any calcium and magnesium fatty acid soaps which may be present.

Fatty Acid Soap

B

The mahogany causes the alkali solution to wet the greasy soil more rapidly, thereby accelerating saponification, and also preserves the tensile strength of the fabric against injury from the relative high concentration of the alkali solution.

Alkali

A

The relatively high concentration of free alkali rapidly attacks saponifiable soil and the soap supplies a latent or reserve supply of alkali as the free alkali is consumed by saponification. The alkali likewise increases the detergency of the fatty acid soap.

Materials

Functions

The fabrics washed with this detergent are cleansed in substantially one-half the usual time, are washed much cleaner and require less rinsing than usual, have no spots or markings from insoluble calcium or magnesium soaps when hardwater is employed, do not tend to become gray upon repeated washings, and do not tend to lose tensile strength at more than one-half the usual rate.

Result

INVENTOR.

Warren T. Reddish

BY

Wood + Wood  
ATTORNEYS.

## UNITED STATES PATENT OFFICE

2,060,529

METHOD OF REMOVING SERICIN FROM  
SILK

Warren T. Reddish, Cincinnati, Ohio, assignor to  
Emery Industries, Inc., Cincinnati, Ohio, a cor-  
poration of Ohio

Original application September 21, 1933, Serial  
No. 690,390. Divided and this application June  
25, 1934, Serial No. 732,389

5 Claims. (Cl. 8—2)

This invention relates to a new detergent adapted for a multitude of processes such as home laundry use, power laundry use, degumming silk, scouring wool, or washing textiles of any nature 5 at any time during the progress of their fabrication and finishing.

The invention can be best explained and understood when presented as an improvement over the subject matter of the British Patent No. 10 19,759, 1912, granted to Grigori Petroff, chemist, of Kuskowo, Russia. This patent refers to and must be read in the light of its companion Patent 15 No. 19,676 of 1912. The patent in question is entitled—"An improved process for manufacturing detergents, detergent solutions, or emulsions". The disclosure of this patent is admirably summarized in the first two claims, which read as follows:

"1. A process for manufacturing a detergent 20 which consists in employing the sulphonic acids extracted by means of alcohol or acetone or like solvents from sulphonated mineral oil hydrocarbons according to the process of Specification No. 19,676 of 1912 as the raw material for producing 25 the detergent.

"2. A process according to claim 1, for manufacturing a detergent which consists in treating the sulphonic acids either in a pure state or in admixture with fats, fatty oils, or fatty acids with 30 caustic or carbonated alkalies or ammonia to obtain a neutral, acid, or alkaline detergent mixture as desired."

The specification, as well as the claims, abounds 35 in the use of the disjunctive and from this it may be inferred that Petroff had gone only so far as to ascertain that his sulphonates were an appropriate raw material to be used as a soap, but that he had not made any determination of how the sulphonates should be used. The most that Petroff 40 claimed for his sulphonate is as follows:

"In regard to its detergent powers, it is in no way inferior to good brands of soap made from fat."

However, though more than twenty years has 45 elapsed since Petroff's work and disclosure, Petroff's novel raw material has never been used either as soap or as an ingredient of soap. This raw material has however been sold to the soap makers all over the world in tremendous quantities and has been used by them in the making of soap as a substitute for the well-known Twitchell reagent for the purpose of splitting fatty glycerides into fatty acids and glycerine. These circumstances conclusively establish the 50 fact that either Petroff was mistaken in his no-

tion or hope that his new raw material was an appropriate ingredient for soap, or that the utilization of his raw material as a soap ingredient was entirely beyond the skill of the soap makers all over the world.

The present invention comprises the selection of ingredients for a detergent including Petroff's raw material and the proportioning of them to provide a detergent far superior to those known in the past. More specifically, the detergent of this invention comprises alkali, fatty acids, and Petroff's mineral oil sulphonics, or mahogany sulphonates, as they are known in this country at the present time. While all of these materials are conventional ones in almost all soap factories, 15 and while all of them have been used as detergents or suggested for use as detergents, still their specific functional relationships have never been understood. On this account they have never been used in combination in practice and in view 20 of the liberal use of the disjunctive in the Petroff disclosure, it cannot be said that they have even been suggested in combination. This functional relationship of alkali, fatty acid soap and mahogany sulphonates is so complex that it is only 25 susceptible to explanation by diagram.

The accompanying drawing is a diagram disclosing how alkali, fatty acid soap and mahogany sulphonates, when used conjointly as a detergent, produce a new and superior detergent 30 result by virtue of the fact that each ingredient in combination with each other ingredient provides a function not provided by any ingredient alone.

Anyone of a number of different alkalies may 35 be employed, such as caustic soda, soda ash, bicarbonate of soda, sodium metasilicate or trisodiumphosphate.

Instead of the sodium compounds of the type listed, the potassium compounds may be employed 40 wherever warranted as a matter of cost. Now, one of the distinguishing characteristics of this invention is that alkali is used for textile washing or treating in much greater quantities and at much higher concentrations than accepted standard practice. Of course, the quantity of alkali used in standard practice varies in different industries according to the nature of the specific problem and even varies among the different plants in a given industry. However, the alkalinity incorporated in this new detergent substantially exceeds previous practice for each use. One reason that the greater strength of alkali can be used without injury to the fabric is that the mahogany sulphonates employed herein seem to act 45 50 55

as inhibitors in relation to the alkali and tend to preserve the tensile strength of the fabric during the washing process.

In contrast to the British Petroff patent, which 5 specifies that the sulphonate may be acid, alkali or neutral, the present detergent is characterized by the presence of a very substantial and ponderable quantity of free alkali or potential alkali of the nature disclosed. For instance, silk is easily 10 injured by alkali and the quantity of alkali used for degumming silk is therefore substantially less than that employed for most of the washing processes. However, even for degumming silk the detergent of this invention comprises at least 5% 15 by weight of a very strong alkali, such as caustic soda. It is therefore to be noted that the detergent of this invention, even at its lower limit of alkalinity, carries a percentage of free alkali which distinguishes it from that lesser degree of 20 alkalinity which is substantially equivalent in operation to neutral or acid solution.

In other words, Petroff specifies that his acid, neutral or alkaline soaps and soap solutions are functionally equivalent and specifies that his 25 starting material, sulphonic acids, optionally mixed with fatty acids, may be neutralized, under-neutralized or over-neutralized without affecting the detergent properties of the resulting soap.

This invention on the contrary is characterized 30 by the presence of anywhere from one-third to twenty times the quantity of alkali necessary to neutralize the mahogany sulphonic and fatty acid content of the admixture. This detergent is not functionally equivalent to an acid or neutral 35 detergent or to an over-neutralized detergent, but on the contrary its detergent action may be said to be dominated by the activity of the large quantity of free or potential alkali.

The fatty acid soap employed in this detergent 40 may be of animal or vegetable origin and of any titre, the soap from fatty acids having a titre as low as ten having been found entirely satisfactory. Red oil soap is entirely suitable for use in this detergent, though soaps from high titre fats, 45 either alone or in combination with red oil soap, may be used.

One of the essential ingredients of the detergent of this invention is mahogany sulphonates. 50 These bodies are produced in the refining of petroleum or fractions thereof, such as lubricating stock, into medicinal white oil or the light colored technical oils. In this general process the petroleum is treated with fuming sulphuric acid or sulphur trioxide, after which the sludge settles 55 out. Next, the oil is treated with an alkali and an aqueous alcohol solution which extracts the mahogany sulphonates, leaving the white oil or light colored technical oil as a remainder.

Mahogany sulphonates are recovered from the 60 aqueous alcoholic solution by evaporation. This general process has frequently been referred to in the patent literature as the Petroff-Humphrey process for the reason that it is practiced under Petroff Patent No. 1,087,888 and Humphrey Patent No. 1,286,179.

There are other variations of this general process, though all of them produce sulphonic bodies which commercially are called mahogany sulphonates. Though these bodies are usually available 70 in the form of the sodium salt of mahogany sulphonic acids, other water soluble salts such as the potassium salt may be used instead of the sodium salt when desired.

While the fatty acid soap and the mahogany 75 sulphonate may be blended and mixed in practi-

cally any ratio according to the specific use for which the detergent is intended, it is recommended that the practice of using 10 to 60% mahogany sulphonates and 90 to 40% fatty acid soap, be followed. These limits were selected arbitrarily, and while not highly critical, are provided for the purpose of instructing the skilled in the art as to the general optimum blending ratio.

As shown in the accompanying drawing, the idea of this invention is to attack the soil on the fabrics or the sericin on raw silk or the wool grease on raw wool or the dressings used on textiles for lubrication or preservation in the course of their manufacture, with a powerful alkali.

The strong free alkali in solution attacks the saponifiable dirt and as it is used up by saponification, the fatty acid soap hydrolyzes and supplies additional alkali (if necessary). The amount of alkali used likewise increases the detergency of the fatty acid soap-mahogany sulphonate mixture. Mahogany sulphonates do not hydrolyze. The fatty acid soap performs another function in conjunction with the mahogany sulphonates. Together they form a body which, in aqueous solution, has more power of suspending and emulsifying dirt, grease, wax and soil in general than does either one of them alone. Mahogany sulphonates from American petroleums do not in general form water soluble calcium and magnesium salts. However, these sulphonates in combination with fatty acid soap do possess the property of solubilizing calcium and magnesium fatty acid soaps or mahogany sulphonates which may be formed as the result of hardness in the water employed for the washing process. This is of very great advantage and it has not been known before that the mixture of mahogany sulphonates and fatty acid soap would emulsify or suspend the calcium or magnesium salts.

The mahogany sulphonates and alkali in combination effect the removal of foreign matter from the textile or fibre being washed without injury to the fibre. The mahogany sulphonates are themselves powerful emulsifying agents even for mineral oil. The combination of mahogany sulphonates and of fatty acid soap, suspends all types of dirt admirably.

The mahogany sulphonates accelerate the wetting out action of the detergent solution and also depress the interfacial tension between the 50 alkaline solution and all oily, greasy or waxy soil or foreign matter on the fabric. Moreover, as before stated, the mahogany sulphonates seem to alter the speed with which the alkali attacks the soil or foreign matter as compared with the 55 speed with which the alkali attacks the textile fibre itself. This action is herein termed an inhibiting action and is a very great advantage, especially in regard to silk or wool, both of which are sensitive to alkalis.

It is therefore to be observed that the use of this detergent for purposes of the type specified provides a very rapid cleansing operation which saves usually one-half of the time normally consumed. In power laundry work the 65 total amount of water used is reduced substantially in half. The clothes are washed much cleaner than is usual, do not tend to become gray on repeated washings, and do not become specked with traces of insoluble calcium and magnesium 70 salts when there is hardness in the water. Moreover, the tensile strength of the fabric being cleansed does not seem to suffer to the extent it does in the processes now used, or to the extent to be expected from the increased amount of al- 75

kali. For instance, garments sent through the usual power laundry fifteen times usually suffer a twelve to fifteen percent loss of tensile strength. Similar garments sent through a similar power laundry using the detergent of this invention seem to lose tensile strength at less than one-half of this rate and in a number of instances have shown only about four percent loss of tensile strength.

10 In summary, it is asserted that the detergent of this invention washes fabrics cleaner and more thoroughly than detergents previously used with less injury to the fabrics and moreover that it reduces the washing time and the consumption 15 of materials, particularly water which is one of the large elements of expense in power laundry practice.

While it is possible to add the ingredients to the washing bath or textile treating bath separately, it is recommended that for most purposes, particularly for power laundry use, the ingredients be pre-combined and thoroughly admixed. In regard to the power laundry use, for instance, the ingredients when admixed in the 25 appropriate proportions, provide a detergent which can be used in finely divided, powdered or granulated form so that it dissolves readily in the washer. Mahogany sulphonates and particularly mahogany sulphonates commercially available in this country, are thick, gummy, sticky bodies, very difficult to handle, pour, measure or remove from shipping containers. The fatty acid soaps and mahogany sulphonates mixed are a viscous jell-like mass, difficult to handle. If, 30 however, two, three, five or more times the amount of dry alkali salt, such as sodium carbonate, be mixed with the mahogany sulphonates and the fatty acid soap, then the detergent becomes a hard, dry body which can be reduced 35 to finely divided or powdered form and readily shipped, handled and measured. It is recommended that the alkali be three to five times the weight of the soap-sulphonate admixture.

While the preferred process of constituting this 45 detergent is reserved for a future application, the proportioning of ingredients to provide the finely divided detergent, as distinguished from a jell-like detergent, is an important element of this invention. The invention and its many specific 50 advantages can be best understood in relation to the following examples of specific uses of the detergent.

#### Laundry practice

55 In modern laundry practice the detergents used consist of high titre fatty acid soaps and alkalis. The ratio of soap to alkali and the type of alkali used varies to some extent in different plants and also depending upon the type 60 of soil to be removed. Ordinarily a ratio of one part of soap to one part of an alkali, consisting of sodium carbonate or a mixture of sodium carbonates and bicarbonate or sodium silicate or sodium phosphate, has been found to give the most satisfactory results.

65 It has also been found that a preliminary treatment of cold water and alkali and possibly a small amount of soap, usually termed a "break" followed by a number of separate sudsing operations produces a greater detergent action for a given amount of fatty soap and alkali than if the same quantity of soap and alkali is used 70 in one sudsing operation. The actual washing operations are followed by a chlorine bleach (in 75 the case of white work) a sufficient number of

rinses to remove the last traces of soaps, a treatment with a mild acid termed the sour to remove the last traces of soaps and alkali and finally a bluing and sizing operation to improve the appearance and finish of the washed materials.

The use of a number of sudsing operations results in improved quality but only at the expense of time of treatment and quantity of water required.

10 We have found that the properties of a detergent comprising a blend of fatty acid soaps and mahogany sulphonates are so different from the ordinary fatty acid soaps that an entirely different washing procedure which results in a 15 material saving in time and water may be employed.

This detergent is also most effective when used with much greater quantities of alkalies than have been found to be the most effective with 20 ordinary fatty acid soaps. A quantity of alkali three to four times greater than that ordinarily used in laundry operations may be used without damage to the material and as a matter of fact on the average the loss in tensile strength is less 25 than with the ordinary laundry procedure and formula.

We have found that a ratio of one part of a blend of 80% of 32 titre fatty acid soap—20% 30 commercial mahogany sulphonate and four parts of soda ash may be used, but one sudsing operation is required to produce work as clean if not cleaner than that produced by a multiple sudsing treatment with fatty acid soap and alkali. The 35 number and duration of the rinses may be reduced as the detergent rinses out very easily.

The following example showing the procedure followed in washing a 250 pound load of household wash work with the fatty acid sulphonate alkali detergent as compared with fatty acid 40 soap and alkali will illustrate the utility and economy of this detergent.

|                            | Fatty acid soap sulphonate and alkali                             | Fatty acid and alkali                         | 45 |
|----------------------------|-------------------------------------------------------------------|-----------------------------------------------|----|
| Wt. of load.....           | 250#                                                              | 250#                                          |    |
| Break.....                 | 12 minutes.                                                       | None.                                         |    |
| First suds.....            | 10 minutes.                                                       | 10 minutes.                                   |    |
| Second suds.....           | None.                                                             | Do.                                           |    |
| Third suds.....            | do.....                                                           | Do.                                           |    |
| Fourth suds.....           | do.....                                                           | Do.                                           |    |
| Fifth suds and bleach..... | do.....                                                           | Do.                                           |    |
| Bleach.....                | 10 minutes.                                                       |                                               |    |
| Rinses.....                | 4-4 min. rinses.                                                  | 5-5 min. rinses.                              |    |
| Sour.....                  | 5 minutes                                                         | 5 minutes.                                    |    |
| Blue.....                  | do.....                                                           | Do.                                           |    |
| Total time.....            | 58 minutes.                                                       | 85 minutes.                                   |    |
| Detergent.....             | 1# 80% fatty acid.....<br>20% sulphonate.....<br>4# soda ash..... | 25# high titre soap.....<br>25# soda ash..... | 55 |

One badly soiled article was torn in two and half run in each load. At the completion of the 60 washing operation it was found that the piece washed with the fatty acid and sulphonate was 2% whiter than the piece washed with fatty soap and alkali.

#### Silk degumming

65 Raw silk consists of the true silk or fibroin covered by a coating of silk gum or sericin. The latter is harsh, non-lustrous and somewhat unstable and must be removed in order that the fibroin may be utilized.

70 Sericin is attacked and rendered partially water soluble by mild alkaline solutions. This property is utilized in removing silk gum, neutral fatty acid soaps in fairly high concentrations (1 to 2%) are most commonly used both as a source 75

of alkali, which is produced by the hydrolysis of the fatty acid soaps in water solution, and as emulsifying and dispersing agents to hold the partially solubilized sericin in solution. Fatty acid soaps are a rather expensive source of alkali and recently small amounts of alkali have been added to the degumming baths in an effort to decrease the amount of soap required and to increase the rate of degumming. Extreme care is required in case excess alkali is used as the fibroin is also attacked by too long an exposure to alkaline solutions or by too high concentrations.

The minimum soap concentration which has been successfully employed in silk degumming is approximately 1.25% and the maximum excess alkali concentration .03%. Attempts to effect a further reduction in soap concentration or an increase in free alkalinity result either in deposition of sericin in the degumming baths or serious weakening of the silk.

By utilizing an emulsifying and detergent mixture comprising a mixture of from 50 to 85 parts of sodium oleate and 50 to 15 parts of mahogany sulphonate, the concentration of the detergent in the degumming bath may be reduced to as low as .75% and the concentration of the alkali increased to as high as .065% without injury to the silk.

30 The following examples showing the procedure and concentrations used in degumming with red oil soap and with a blend of red oil soap and sulphonate illustrate the advantages of the fatty soap sulphonate detergent.

35

|                                | Fatty soap—sulphonate                                            | Fatty soap              |
|--------------------------------|------------------------------------------------------------------|-------------------------|
| 40 Ratio silk to solution..... | 1 to 50.<br>75% of 70% red oil soap.<br>30% mahogany sulphonate. | 1 to 50.<br>1.25%.      |
| Detergent concentration.....   |                                                                  | .3 gram NaOH per liter. |
| Alkali concentration.....      | .65 gram NaOH per liter.                                         | Just below boil.        |
| Temperature.....               | Just below boil.                                                 | Just below boil.        |
| Time.....                      | 45 minutes.                                                      | 45 minutes.             |
| 45 Boil-off loss.....          | 23.1                                                             | 23.3.                   |

From the above results it will be seen that the amount of detergent can be reduced by 40% without any increases in time of degumming and 50 without weakening of the silk.

If the concentration of the red oil sulphonate mixture is increased to 1.25% the time may be reduced to 30 minutes, resulting in a saving in time of 33 1/3 per cent.

#### Treatment of wool

Wool is treated with detergent solutions either alone or in conjunction with alkalies several 60 times in the course of manufacture. Raw wool is contaminated by dirt and earthy matter, wool grease and suint all of which must be removed to render the wool suitable for further manufacturing operations. The oils which are added to 65 facilitate the spinning and weaving operations must be removed prior to dyeing which necessitates a second scouring operation. In the fulling operation which is carried out as a part of the final finishing operation, detergent solutions and alkalies are also used.

70 Wool is quite sensitive to the action of alkalies and care must be exercised in using alkalies in the scouring baths. It is also necessary to employ moderate temperatures, preferably not over

140° F. as higher temperatures cause harshening and deteriorate the fibres.

The amount of soap and the ratio of soap to alkali used in scouring raw wool varies widely depending upon the character of the wool and 5 the nature and amount of impurities associated with it, from .25% to 1.25% soap and from 1.25 to 2.5% of soda ash being used. The relatively high soda ash content serves to saponify fatty acids which may be present as constituents of 10 the wool grease.

In scouring woven fabrics for removal of the oils used in manufacture from 1.5 to 5% soap and from .5 to 2.5% of soda ash may be used, the preferred amounts depending upon the quantity 15 of spinning oils present and their content of saponifiable constituents.

In fulling approximately the same strength soap solutions are used but the alkali used is generally reduced. Alkali is necessary to exert a 20 softening and swelling action and to accelerate the shrinkage and felting which occurs during the fulling operation.

If in place of fatty acid soap a blend of from 50 to 85% of fatty acid soap and from 15 to 50% 25 mahogany sulphonate is used the quantity of alkali used in the baths may be greatly increased without affecting the strength of the wool or harshening it or affecting its dyeing properties.

In scouring raw wool the amount of alkali may 30 be doubled and the amount of detergent decreased, the high emulsifying power of the fatty soap sulphonate blend in the presence of an appreciable alkali concentration will exert a wetting out, cleansing and soil dispersing action even 35 when present in a reduced amount.

In scouring piece-goods, the time of scouring and the quantity of detergent may be decreased if the mineral sulphonate fatty soap blend is used. In case the spinning oils have a high 40 mineral oil content it is preferable to use a higher proportion of mahogany sulphonate in the detergent blend.

The alkali content of the fulling baths may be increased and the fulling time reduced by increasing the alkali content. In the presence of the mahogany sulphonate and fatty detergent, the wool is not harshened and the wetting and penetrating powers of the solution are enhanced.

The following example illustrates the use of 50 the mahogany sulphonate fatty soap blend as compared to the fatty soaps commonly used in scouring woolen piece-goods.

|                              | Fatty soap—sulphonate                | Fatty soap                                          |
|------------------------------|--------------------------------------|-----------------------------------------------------|
| Ratio wool to solution.....  | 1 to 6.<br>80%—35 titre fatty acids. | 1 to 6.<br>3 oz. per gal.<br>palm and red oil soap. |
| Detergent—2 oz. per gal..... | 5 oz. per gal.                       | 35 titre.<br>20% mahogany sulphonate.<br>soda ash.  |
| Temperature.....             | 120° F.                              | 120° F.                                             |
| Time.....                    | 35 min.                              | 45 min.                                             |

65 The color, appearance and softness of the material scoured with the fatty soap sulphonate mix were equal in all respects to the material scoured with fatty soaps, although the scouring time was reduced approximately 20%, approximately one-third less of the fatty acid sulphonate mix than fatty soap was used.

70 This application is divisional of my co-pending application Serial No. 690,390, filed September 21, 1933.

75

Having described my invention, what I claim is:

- 5 1. The method of removing sericin from raw silk, which comprises, treating the silk bearing the sericin in a hot aqueous solution containing mahogany sulphonates, water soluble fatty acid soap, and caustic soda, the quantity of caustic soda employed equaling at least 5% by weight of the soap-sulphonate admixture.
- 10 2. A raw silk degumming process, comprising, treating the raw silk in a hot aqueous bath comprising mahogany sulphonates in admixture with water soluble fatty acid soap, and alkali, said alkali content being at least 5% by weight of the sulphonate soap mixture.
- 15 3. A raw silk degumming process, comprising, treating the raw silk in a hot aqueous bath comprising, mahogany sulphonates in admixture with water soluble fatty acid soap, and an alkali salt adapted when dissolved in water to yield a free alkali.
4. A process of removing sericin from raw silk, said process, comprising, treating the raw sericin bearing silk with a detergent in a hot aqueous solution, said detergent comprising 50 to 15% mahogany sulphonates, 50 to 85% water soluble fatty acid soap, and a quantity of an alkaline salt adapted to yield free alkali to the extent of at least 5% by weight of the soap sulphonate mixture.
- 10 5. A solution adapted for use in degumming raw silk in the ratio of 50 parts of solution to one part raw silk, said solution characterized by a detergent concentration of 0.75 %, said detergent comprising water soluble fatty acid soap and mahogany sulphonate, and a free alkali concentration of 0.65 gram NaOH per liter.

WARREN T. REDDISH.